

## UNITED STATES PATENT OFFICE

WILLIAM CLARENCE LODGE, OF FULTON, NEW YORK, ASSIGNOR TO OSWEGO FALLS CORPORATION, OF FULTON, NEW YORK, A CORPORATION OF NEW YORK

## PAPER PRODUCT AND METHOD OF PRODUCING THE SAME

No Drawing.

Application filed January 28, 1927. Serial No. 164,382.

The object of this invention is to produce paper products of maximum strength while possessing maximum water resisting qualities, and also to produce such products of substantial strength and water resistant qualities without substantial increase in production costs.

Primarily with the foregoing object in view, I have discovered that paper products where sizing is added during the paper making process, attain economy in production combined with approximately maximum (a) strength, and (b) water resistance qualities, when the product contains not more than approximately one percent wax or its equivalent, and not more than approximately three percent rosin or its equivalent; and that the preferred method of producing such paper product is to add to the pulp in the beater during the paper making process, as a sizing, (1) an emulsion or suspension of rosin or equivalent ingredient equal by weight to approximately three percent of the pulp and then (2) an emulsion or suspension of paraffin or equivalent water resisting agent or ingredient equal by weight to approximately one percent of the pulp, and thereafter add to the pulp in the beater a proportion of suitable fixing or precipitating agent, such as alum or its equivalent, equal by weight to approximately three percent of the pulp.

By the term "paper products", I include paper or paper board in the sheet or roll, and also paper articles, such as paper containers of various forms, and paper closures, such as paper closure disks and paper hood caps, for bottles and other containers.

While it is highly desirable to provide paper containers and paper closures, the paper or paper board of which is approximately water proof or of good water resistant qualities, yet it is exceedingly disadvantageous to provide paper products of substantially weak paper material, wherein the strength of the paper is substantially weakened as the water resistant quality of the paper is increased, and it is also objectionable to substantially increase paper production costs by reason of the attainment of substantial water resistant qualities in the paper product.

It is highly desirable that paper hood caps (paper caps of skirted form designed to cover and protect the heads of containers, particularly milk bottles) be of more or less high tensile strength, and possess substantial water resistant qualities, and where such hood caps carry a binder rendering the caps moldable when heated and quick setting to rigid securing form, it is particularly desirable that the caps possess the qualities of strength as well as resistance against the entrance of moisture and consequent swelling of the paper material with a tendency to expand and unduly loosen the binder carrying skirt molded on the bottle neck.

In making my tests under this invention, I have followed sizing methods in the production of paper or paper board, particularly that grade of paper board commonly known as "manilla sulphite" or "oyster pail", and hood caps for bottles, made from such board.

It is known to those skilled in the art, that waxes and fats generally, and paraffin specifically, materially improve the water resistance of paper and paper products when incorporated into the sheet of paper either by the process commonly known as "engine sizing" in which process a solution, emulsion or finely dispersed suspension of wax or waxes alone or in combination with rosin and/or other ingredients, is added to the paper pulp in the beaters; or when the wax is applied to a surface of the finished sheet of paper by immersion in a bath of molten wax, or by any other convenient method.

However, I find that the addition of any of these sizing materials and/or compounds to the paper pulp in the beater, has a marked weakening effect on the tensile strength of the finished sheet or paper product.

I have tested paper products the pulp for which was subjected to various engine sizing treatments during the paper making process, and in the following tables I have tabulated various results attained and compared the same with the results attained with paper products of and produced according to, my invention.

In the following tables, and explanations, the percentage or proportion of size added to

the pulp, indicates approximately the amount of sizing material in the finished sheet or paper product independent of the concentration of the emulsion or suspension of the size as introduced.

5 "Paraffin" in the following tables means an aqueous emulsion or suspension containing substantially pure paraffin wax as the only sizing agent in the preparation.

10 "50-50 paraffin and rosin", hereinafter means that approximately equal weights of rosin and paraffin wax were fused and then emulsified or finely dispersed in water.

15 "Rosin" hereinafter means the ordinary rosin size of commerce, that is a solution of sodium resinate containing more or less "free" or unsaponified rosin, (in this instance 30% of the total rosin present).

20 As to the tensile strength of variously sized finished paper, my tests show as follows, an unsized sheet of paper board being used as a standard:

| 25 | (1) Size added              | Strength | Decrease    |
|----|-----------------------------|----------|-------------|
|    |                             |          | in Strength |
|    | None                        | 100%     |             |
|    | 1% paraffin                 | 90%      | 10%         |
|    | 5% paraffin                 | 75%      | 25%         |
|    | 2% 50-50 paraffin and rosin | 60%      | 40%         |
|    | 5% 50-50 paraffin and rosin | 50%      | 50%         |
| 30 | 1% paraffin and 2% rosin    | 85%      | 15%         |
|    | 1% paraffin and 3% rosin    | 80%      | 20%         |
|    | 2% paraffin and 2% rosin    | 75%      | 25%         |

35 I find that paraffin wax has a weakening effect on the strength of the sheet, that this effect increases with the amount added, although not in exact proportion to it. I also find by blending wax and rosin together and then emulsifying the resultant mixture that a compound is formed which exerts proportionately a greater effect on the strength of the finished sheet than paraffin alone.

40 (2) I find the sizing efficiency of the various mixtures is not in proportion to their amount or composition. The effect of these various mixtures on the water resistance of the paper in which they are used is tabulated below and the results are expressed as percent of water absorbed by sheets of uniform thickness when submerged in distilled water at a 45 temperature plus or minus 70° Fahrenheit for exactly twenty minutes.

| 55 | Size added                  | Percent moisture absorbed | 35 |
|----|-----------------------------|---------------------------|----|
|    |                             |                           |    |
|    | 1% paraffin                 |                           | 24 |
|    | 5% paraffin                 |                           | 38 |
|    | 2% 50-50 paraffin and rosin |                           | 28 |
|    | 5% 50-50 paraffin and rosin |                           | 28 |
|    | 1% paraffin and 2% rosin    |                           | 28 |
|    | 1% paraffin and 3% rosin    |                           | 24 |
| 60 | 2% paraffin and 2% rosin    |                           | 28 |
|    | 3% rosin                    |                           | 75 |

65 I find that while rosin of itself is very inferior to wax alone, that the combination of the rosin with the wax materially improves

the sizing properties of the rosin, so much so that approximately 1% of wax in the finished sheet is sufficient for all practical purposes and may be taken as the optimum amount.

70

I find that greater efficiency is obtained by the use of separately prepared emulsions or suspensions of rosin and wax. It is also observed that this method produces a stronger finished product than any of the others enumerated.

75

(3) I find that when wax and rosin are used in this way, the retention of the rosin is materially improved, for example: To 1000 pounds of pulp in the beater is added 30 pounds of rosin as emulsified size followed after an interval of ten minutes by 30 pounds of alum, the stuff passed through a Jordan engine and formed into board on a cylinder machine.

80

The finished board contained 2% of resinous material of which 1.2% was present in the original pulp, leaving .8% which has been absorbed in the size, showing a retention of

85

.8  
3.0 or 26%

The process was repeated with the addition of 10 pounds of emulsified paraffin wax added immediately after the rosin size and before the addition of the alum. The finished board was found on analysis to contain .95% paraffin and 3.9% of resinous material, of which 1.2% was present in the original pulp as before, leaving 2.7% which had been absorbed—the size thus showing a retention of

90

2.7  
3.0 or 90%

100 These results were obtained in commercial production. The pulp was less than one hour in the beater, and the board made on a six cylinder machine.

105

110 Any substance that will form soluble soap with an alkali, for paper sizing purposes, such as stearic acid, stearine, and many vegetable and animal fats, could be used as a substitute for rosin, for the purposes of my invention, in paper sizing, and hence the term "sizing soap" 115 employed herein to include rosin and its substitutes for sizing purposes within my invention. However, rosin is at this time preferable because it can be readily obtained in the desired quantities at a reasonable price.

115

120 Various substances or compounds can be substituted for paraffin to perform the functions of paraffin within my invention. Any substance that will perform the functions of paraffin under my invention and that is susceptible of emulsification, or that will exist in a fine state of subdivision, in an aqueous menstruum, can be substituted for paraffin, for instance, ceresin, Montan, carnauba, and Japan wax, beeswax, asphalt emulsions, and emulsions of oils and/or fats, the latter as distin-

125

130

guished from the soluble soaps that include rosin. Under my invention, paraffin may be replaced by one of these paraffin substitutes or mixtures of two or more thereof, but such 5 substitutes may or may not be as efficient, and/or economical, pound for pound, as paraffin. As at present advised by experience and market conditions, I prefer to employ paraffin, or mixtures of paraffin and carnauba or Montan waxes, with rosin.

10. Where the paper product of my invention will be exposed to heat, say above the melting point of paraffin, carnauba, or Montan wax or asphalt would be preferable to paraffin, but 15 on the other hand, the color of some of these paraffin substitutes might be objectionable in paper products, for some purposes.

What I claim is:—

1. In the production of a water resistant 20 paper product, those steps which consist in adding to the pulp in the paper making process, approximately 2% to 3% sizing soap such as rosin, and approximately 1% water resistant ingredient as a sizing, and fixing or precipitating said sizing in the pulp.

2. In the production of a water resistant 30 paper product, those steps which consist in adding to the pulp, sizing in the proportion of three parts rosin or rosin substitute and approximately one part wax or wax substitute, and thereafter fixing or precipitating the same in the pulp, for the final production of paper product containing approximately 1% wax and not more than 3% rosin.

35. In testimony whereof I have hereunto set my hand at Fulton, New York, this 27th day of Jan., 1927.

WM. C. LODGE.

40

45

50

55

60